

3,421,888

## COPPER ALLOY

Matti J. Saarivirta, Marquette, Mich., assignor, by mesne assignments, to Calumet & Hecla Corporation, Evanston, Ill., a corporation of Delaware  
No Drawing. Filed Aug. 12, 1966, Ser. No. 571,983  
U.S. Cl. 75—159 3 Claims  
Int. Cl. C22c 9/00

This invention relates to a copper base alloy having good responses to precipitation hardening and cold working.

Copper alloys of high tensile strength, hardness and good electrical conductivity are well known in the art. Thus, alloys of this type are the copper-beryllium alloys and particularly copper-beryllium-cobalt alloys. These, however, are expensive so that the cost limits their use.

One of the features of this invention is to provide a copper base alloy having good responses to precipitation hardening and cold working to produce an alloy of high tensile strength, good electrical conductivity and excellent hardness that is considerably cheaper than previous alloys having these characteristics, the new alloy containing, by weight, about 0.4-1.5% chromium, about 0.3-0.9% titanium, about 0.1-0.8% nickel, about 0.02-0.16% phosphorus, the remainder being substantially oxygen free copper, in which the weight amount ratio of nickel to phosphorus is about 5 of nickel to 1 of phosphorus and the weight amount of titanium is about 1-1.7 times the sum of the amounts of nickel plus phosphorus.

The copper of the alloy contains the lowest amount possible of oxygen. This can be either initially oxygen free copper which is ordinarily produced in a reducing atmosphere, an inert atmosphere or a vacuum or it can be copper that has been deoxidized with such well known deoxidizers as phosphorus, silicon, lithium, calcium, calcium boride or the like which combine with the oxygen in the copper to eliminate it substantially completely.

The alloys of this invention have been found to be useful in manufacturing resistance welding electrodes as well as electrical and electronic components generally.

The presence of the chromium in the alloy increases the response of the alloy to precipitation hardening and gives increased hardness and tensile strength. The titanium also appears to increase the hardness of the alloy.

The new alloy may be fully annealed by solution heat treatment in a non-oxidizing atmosphere, either reducing or inert. This is a well known procedure in which the alloy is heated to a temperature between about 900-1000° C. and then cooled by rapid quenching. The solution heat treated alloy of this invention responds excellently to precipitation or age hardening. This is generally done by reheating the quenched alloy for one hour or more at about 300-600° C. for the generally one or more hours of aging. In general, the higher the temperature of heating the shorter the aging time. In practice excellent precipitation hardening conditions have been to reheat to about 500° C. for about 2 hours. Such precipitation hardening strengthens the alloy while at the same time increasing the thermal and electrical conductivity.

The strength and hardness of the alloy can be further increased by the customary cold working which is performed in the usual manner. This cold working may be an intermediate step between the solution heat treatment and the precipitation hardening or it may be done after precipitation hardening, as desired.

Thus the copper-chromium-titanium-nickel-phosphorus alloys of this invention are highly precipitation hardenable and give excellent response to cold working. Heat treatment at 500° C. after solution annealing at 1020° C. results in an ultimate tensile strength of 80,000-83,000 p.s.i., 77-83 Rockwell B hardness and 55-65% IACS

electrical conductivity. When cold worked to a 15% reduction in area, the tensile strength is 90,000-97,000 p.s.i., hardness 88-92 and the electrical conductivity is not changed. Very similar properties are obtained by solution annealing, 60% cold reduction and heat treating. The new alloys can be easily melted and cast without difficulty providing the usual protective atmosphere is maintained.

The following tables set forth various alloys coming within the invention, their treatments and their properties. In each example the copper was melted first, then the chromium added and completely dissolved in the copper melt, then the titanium dissolved in the copper melt and finally the nickel and phosphorus added and the entire molten alloy mixed to a homogeneous condition. 500-1000 gram castings were then made at casting temperatures of 1110-1200° C. in graphite and cast iron molds with each 1000 gram casting being about 0.75 inch in diameter by 12 inches long and the 500 gram castings being about 0.75 inch in diameter by 6 inches long. During the melting and the casting the melts were maintained under non-oxidizing conditions in that they were surrounded by an atmosphere of an inert gas, with argon being especially preferred for this purpose.

The following tables present various examples of alloys within the invention and their characteristics. Thus, in the following Table No. 1 there is shown the effect of various amounts of nickel and phosphorus forming nickel-phosphide on the properties of basic copper-chromium-titanium alloys. The other tables record the effects of various treatments on the alloys of this invention.

TABLE 1

[Cast specimens solution annealed at 1,020° C. for 30 minutes, quenched, and heat treated at 500° C. for 2 hours]

| Example                                               | Percent |     | Solution annealed                  |                                           | Heat treated                             |                                    |
|-------------------------------------------------------|---------|-----|------------------------------------|-------------------------------------------|------------------------------------------|------------------------------------|
|                                                       | Ni      | P   | Hardness<br>VPN<br>percent<br>IACS | Elec.<br>cond.,<br>VPN<br>percent<br>IACS | Hardness<br>VPN<br>Rb<br>percent<br>IACS | Elec.<br>cond.,<br>percent<br>IACS |
| Copper Alloy Containing 1% Chromium and 0.3% Titanium |         |     |                                    |                                           |                                          |                                    |
| 1.                                                    | .10     | .02 | 46                                 | 31                                        | 140                                      | 77                                 |
| 2.                                                    | .20     | .04 | 47                                 | 28                                        | 145                                      | 79                                 |
| 3.                                                    | .30     | .06 | 45                                 | 29                                        | 140                                      | 77                                 |
| 4.                                                    | .40     | .08 | 46                                 | 30                                        | 136                                      | 76                                 |
| 5.                                                    | .60     | .12 | 51                                 | 25                                        | 145                                      | 75                                 |
| 6.                                                    | .80     | .16 | 51                                 | 28                                        | 136                                      | 71                                 |
| Copper Alloy Containing 1% Chromium and 0.4% Titanium |         |     |                                    |                                           |                                          |                                    |
| 7.                                                    | .10     | .02 | 49                                 | 26                                        | 144                                      | 76                                 |
| 8.                                                    | .20     | .04 | 50                                 | 27                                        | 145                                      | 77                                 |
| 9.                                                    | .30     | .06 | 49                                 | 27                                        | 153                                      | 79                                 |
| 10.                                                   | .40     | .08 | 49                                 | 28                                        | 136                                      | 73                                 |
| 11.                                                   | .60     | .10 | 54                                 | 29                                        | 140                                      | 73                                 |
| Copper Alloy Containing 1% Chromium and 0.5% Titanium |         |     |                                    |                                           |                                          |                                    |
| 12.                                                   | .10     | .02 | 58                                 | 20                                        | 154                                      | 79                                 |
| 13.                                                   | .20     | .04 | 57                                 | 22                                        | 143                                      | 81                                 |
| 14.                                                   | .30     | .06 | 58                                 | 24                                        | 145                                      | 77                                 |
| 15.                                                   | .40     | .08 | 49                                 | 27                                        | 143                                      | 77                                 |
| 16.                                                   | .50     | .10 | 56                                 | 25                                        | 145                                      | 79                                 |
| 17.                                                   | .60     | .12 | 55                                 | 24                                        | 153                                      | 79                                 |
| 18.                                                   | .80     | .16 | 55                                 | 24                                        | 138                                      | 76                                 |
| Copper Alloy Containing 1% Chromium and 0.6% Titanium |         |     |                                    |                                           |                                          |                                    |
| 19.                                                   | .10     | .02 | 54                                 | 19                                        | 149                                      | 80                                 |
| 20.                                                   | .20     | .04 | 53                                 | 24                                        | 139                                      | 80                                 |
| 21.                                                   | .30     | .06 | 54                                 | 25                                        | 155                                      | 80                                 |
| 22.                                                   | .40     | .08 | 53                                 | 22                                        | 148                                      | 80                                 |
| 23.                                                   | .50     | .10 | 53                                 | 26                                        | 150                                      | 79                                 |
| 24.                                                   | .60     | .12 | 50                                 | 25                                        | 150                                      | 78                                 |
| 25.                                                   | .70     | .14 | 55                                 | 25                                        | 148                                      | 78                                 |
| Copper Alloy Containing 1% Chromium and 0.7% Titanium |         |     |                                    |                                           |                                          |                                    |
| 26.                                                   | .10     | .02 | 78                                 | 20                                        | 154                                      | 81                                 |
| 27.                                                   | .20     | .04 | 70                                 | 18                                        | 155                                      | 81                                 |
| 28.                                                   | .30     | .06 | 55                                 | 23                                        | 155                                      | 81                                 |
| 29.                                                   | .40     | .08 | 52                                 | 29                                        | 145                                      | 81                                 |
| 30.                                                   | .50     | .10 | 65                                 | 22                                        | 157                                      | 83                                 |
| 31.                                                   | .60     | .12 | 65                                 | 24                                        | 160                                      | 83                                 |
| 32.                                                   | .70     | .14 | 68                                 | 26                                        | 150                                      | 79                                 |

Copper Alloy Containing 1% Chromium and 0.9% Titanium

|    |     |     |    |    |     |    |    |
|----|-----|-----|----|----|-----|----|----|
| 33 | .10 | .02 | 67 | 15 | 150 | 81 | 24 |
| 34 | .20 | .04 | 74 | 13 | 160 | 85 | 21 |
| 35 | .30 | .06 | 78 | 16 | 152 | 82 | 29 |
| 36 | .40 | .08 | 64 | 16 | 166 | 85 | 30 |
| 37 | .60 | .12 | 99 | 19 | 145 | 81 | 27 |
| 38 | .70 | .14 | 60 | 17 | 160 | 84 | 43 |
| 39 | .80 | .16 | 64 | 23 | 138 | 81 | 55 |

TABLE 2

[Effect of heat treating temperatures on the hardness and electrical conductivity of the Cu-Cr-Ti-Ni-P alloys. The cast specimens were solution annealed at 1,020° C. for 30 minutes, quenched, and heat treated at various temperatures for 2 hours]

| Condition                                                                                        | Hardness |    | Elec. cond., percent IACS |
|--------------------------------------------------------------------------------------------------|----------|----|---------------------------|
|                                                                                                  | VPN      | Rb |                           |
| Example 2.—Copper Alloy Containing 1% Chromium, 0.3% Titanium, 0.2% Nickel and 0.04% Phosphorus  |          |    |                           |
| No aging                                                                                         | 48       | —  | 28                        |
| Aged at 450° C.                                                                                  | 110      | 65 | 59                        |
| Aged at 470° C.                                                                                  | 130      | 74 | 65                        |
| Aged at 500° C.                                                                                  | 145      | 79 | 69                        |
| Aged at 525° C.                                                                                  | 126      | 69 | 69                        |
| Aged at 550° C.                                                                                  | 117      | 64 | 72                        |
| Aged at 650° C.                                                                                  | 83       | 35 | 64                        |
| Aged at 700° C.                                                                                  | 68       | 20 | 60                        |
| Example 29.—Copper Alloy Containing 1% Chromium, 0.7% Titanium, 0.4% Nickel and 0.08% Phosphorus |          |    |                           |
| No aging                                                                                         | 53       | 46 | 29                        |
| Aged at 500° C.                                                                                  | 148      | 81 | 61                        |
| Aged at 550° C.                                                                                  | 122      | 69 | 64                        |
| Aged at 600° C.                                                                                  | 112      | 60 | 60                        |
| Aged at 650° C.                                                                                  | 87       | 40 | 57                        |
| Aged at 700° C.                                                                                  | 74       | 23 | 55                        |

TABLE 3

[Effect of various solution annealing temperatures on the properties of the Cu-Cr-Ti-Ni-P alloys. The cast specimens were solution annealed at the temperatures indicated for 30 minutes, quenched, and aged at 500° C. for 2 hours]

| Alloy      | Temperature, ° C. | Hardness |    | Elec. cond., percent IACS |
|------------|-------------------|----------|----|---------------------------|
|            |                   | VPN      | Rb |                           |
| Example 2  |                   |          |    |                           |
| Example 2  | 900               | 106      | 48 | 71                        |
| Example 8  | 900               | 106      | 61 | 68                        |
| Example 15 | 900               | 107      | 54 | 60                        |
| Example 21 | 900               | 106      | 59 | 62                        |
| Example 29 | 900               | 107      | 59 | 64                        |
| Example 38 | 900               | 124      | 69 | 44                        |
| Example 2  | 925               | 110      | 57 | 71                        |
| Example 8  | 925               | 109      | 61 | 68                        |
| Example 15 | 925               | 108      | 60 | 59                        |
| Example 21 | 925               | 110      | 63 | 61                        |
| Example 29 | 925               | 109      | 63 | 65                        |
| Example 38 | 925               | 129      | 70 | 43                        |
| Example 2  | 950               | 114      | 63 | 72                        |
| Example 8  | 950               | 118      | 66 | 68                        |
| Example 15 | 950               | 117      | 65 | 65                        |
| Example 21 | 950               | 124      | 68 | 62                        |
| Example 29 | 950               | 124      | 67 | 65                        |
| Example 38 | 950               | 134      | 74 | 41                        |
| Example 2  | 975               | 121      | 66 | 71                        |
| Example 8  | 957               | 124      | 71 | 66                        |
| Example 15 | 975               | 124      | 69 | 61                        |
| Example 21 | 975               | 132      | 72 | 62                        |
| Example 29 | 975               | 130      | 72 | 64                        |
| Example 38 | 975               | 144      | 77 | 40                        |
| Example 2  | 1,000             | 125      | 73 | 71                        |
| Example 8  | 1,000             | 134      | 73 | 65                        |
| Example 15 | 1,000             | 134      | 73 | 63                        |
| Example 21 | 1,000             | 134      | 74 | 62                        |
| Example 29 | 1,000             | 136      | 76 | 64                        |
| Example 38 | 1,000             | 144      | 80 | 42                        |
| Example 2  | 1,020             | 145      | 79 | 69                        |
| Example 8  | 1,020             | 145      | 78 | 66                        |
| Example 15 | 1,020             | 140      | 77 | 64                        |
| Example 21 | 1,020             | 157      | 80 | 62                        |
| Example 29 | 1,020             | 148      | 82 | 61                        |
| Example 38 | 1,020             | 160      | 84 | 43                        |
| Example 2  | 1,040             | 143      | 79 | 70                        |
| Example 8  | 1,040             | 140      | 79 | 66                        |
| Example 15 | 1,040             | 142      | 77 | 64                        |
| Example 21 | 1,040             | 147      | 82 | 63                        |
| Example 29 | 1,040             | 146      | 80 | 60                        |
| Example 38 | 1,040             | 143      | 79 | 44                        |

TABLE 4

Effect of cold working after aging. Cast specimens hot forged to 0.45 inch with 50% reduction, solution annealed at 1,020° C. for 30 minutes, quenched, aged at 500° C. for 2 hours and cold worked various amounts in cross section]

| 5  | Alloy  | Solution annealed and aged |    |                           | Cold worked after aging |     |    |                           |
|----|--------|----------------------------|----|---------------------------|-------------------------|-----|----|---------------------------|
|    |        | VPN                        | Rb | Elec. cond., percent IACS | Percent cold reduct.    | VPN | Rb | Elec. cond., percent IACS |
| 10 | Ex. 40 | 146                        | 78 | 58                        | 7                       | 155 | 82 | 57                        |
|    | Ex. 29 | 134                        | 75 | 62                        | 9                       | 164 | 82 | 61                        |
| 15 | Ex. 38 | 155                        | 81 | 49                        | 9                       | 172 | 90 | 49                        |

Example 40—Copper alloy containing 1% chromium, 0.55% titanium, 0.28% nickel and 0.032% phosphorus.

TABLE 5

[Certain properties of the solution annealed, aged and cold drawn Cu-Cr-Ti-Ni-P alloys wires. The 0.128 inch diameter wire was solution annealed at 1,020° C. for 20 minutes, quenched, heat treated at 500° C. for 2 hours, and cold drawn after heat treatment to 0.116 inch with 15% reduction in area]

| 30 | Ex.           | Condition | Tensile strength, p.s.i. | Elong., percent in 2 in. | Hardness |    | Elec. cond., percent IACS |
|----|---------------|-----------|--------------------------|--------------------------|----------|----|---------------------------|
|    |               |           |                          |                          | VPN      | Rb |                           |
| 2  | Sol. annealed | 38,000    | 30                       | 52                       | 47       | 27 |                           |
|    | Aged          | 79,000    | 16                       | 141                      | 75       | 60 |                           |
|    | Cold drawn    | 82,000    | 6                        | 167                      | 85-90    | 60 |                           |
| 9  | Sol. annealed | 43,000    | 30                       | 51                       | 48       | 28 |                           |
|    | Aged          | 82,000    | 13                       | 145                      | 78       | 64 |                           |
|    | Cold drawn    | 90,000    | 5                        | 170                      | 87-90    | 63 |                           |
| 15 | Sol. annealed | 44,000    | 26                       | 51                       | 49       | 24 |                           |
|    | Aged          | 83,000    | 15                       | 149                      | 77       | 58 |                           |
|    | Cold drawn    | 93,000    | 5                        | 180                      | 88-92    | 58 |                           |
| 22 | Sol. annealed | 43,000    | 28                       | 53                       | 51       | 26 |                           |
|    | Aged          | 83,000    | 12                       | 146                      | 79       | 62 |                           |
|    | Cold drawn    | 92,000    | 5                        | 171                      | 88-90    | 60 |                           |
| 29 | Sol. annealed | 43,000    | 23                       | 53                       | 58       | 25 |                           |
|    | Aged          | 80,000    | 13                       | 150                      | 80       | 58 |                           |
|    | Cold drawn    | 96,000    | 5                        | 180                      | 88-92    | 58 |                           |
| 38 | Sol. annealed | 42,000    | 23                       | 51                       | 50       | 21 |                           |
|    | Aged          | 83,000    | 17                       | 155                      | 83       | 50 |                           |
|    | Cold drawn    | 90,000    | 5                        | 183                      | 88-21    | 47 |                           |
| 41 | Sol. annealed | 43,000    | 27                       | 50                       | 45       | 23 |                           |
|    | Aged          | 83,000    | 14                       | 155                      | 81       | 55 |                           |
|    | Cold drawn    | 96,000    | 5                        | 180                      | 88-92    | 55 |                           |

Example 41—Copper alloy containing 1% chromium, 0.7% titanium, 0.4% nickel and 0.08% phosphorus.

| 65 | Example | Percent cold reduct. in cross sect. | Cold worked condition |    | Cold worked and aged      |     |    |    |
|----|---------|-------------------------------------|-----------------------|----|---------------------------|-----|----|----|
|    |         |                                     | VPN                   | Rb | Elec. cond., percent IACS | VPN |    |    |
| 70 | 40      | 16                                  | 78                    | 44 | 25                        | 150 | 80 | 58 |
|    |         | 34                                  | 106                   | 68 | 24                        | 160 | 83 | 60 |
|    |         | 46                                  | 116                   | 61 | 24                        | 170 | 85 | 61 |
| 70 | 38      | 16                                  | 86                    | 51 | 18                        | 155 | 88 | 55 |
|    |         | 34                                  | 112                   | 65 | 20                        | 173 | 89 | 55 |
|    |         | 46                                  | 120                   | 66 | 19                        | 181 | 91 | 55 |

TABLE 7

[Effect of heat treating temperatures on the properties of the cold drawn wires of Cu-Cr-Ti-Ni-P alloys. The 0.128 inch diameter wires were solution annealed at 1,020° C. for 20 minutes, quenched, cold drawn to 0.081 inch with 60% reduction in area and heat treated at various temperatures for 1 hours]

| Example | Condition     | Tensile strength, p.s.i. | Elong., percent in 2 inches | Hardness VPN | Elec. cond., percent IACS |
|---------|---------------|--------------------------|-----------------------------|--------------|---------------------------|
| 2-----  | Cold drawn... | 64,000                   | 3                           | 124          | 26                        |
|         | Aged at:      |                          |                             |              |                           |
|         | 350° C....    | 66,000                   | 4                           | 130          | 32                        |
|         | 400° C....    | 71,000                   | 6                           | 138          | 41                        |
|         | 450° C....    | 85,000                   | 8                           | 168          | 54                        |
|         | 475° C....    |                          | 9                           | 174          | 57                        |
|         | 500° C....    | 90,000                   | 9                           | 169          | 62                        |
|         | 550° C....    | 80,000                   | 10                          | 153          | 60                        |
|         | 600° C....    | 67,000                   | 7                           | 136          | 54                        |
| 9-----  | Cold drawn... | 64,000                   | 3                           | 124          | 26                        |
|         | Aged at:      |                          |                             |              |                           |
|         | 350° C....    | 66,000                   | 3                           | 126          | 32                        |
|         | 400° C....    | 69,000                   | 6                           | 138          | 41                        |
|         | 450° C....    | 83,000                   | 8                           | 170          | 56                        |
|         | 475° C....    | 85,000                   | 8                           | 171          | 61                        |
|         | 500° C....    | 90,000                   | 9                           | 169          | 65                        |
|         | 525° C....    | 85,000                   | 9                           | 165          | 67                        |
|         | 550° C....    | 78,000                   | 8                           | 153          | 67                        |
| 15----- | Cold drawn... | 67,000                   | 3                           | 128          | 23                        |
|         | Aged at:      |                          |                             |              |                           |
|         | 350° C....    | 66,000                   | 4                           | 131          | 28                        |
|         | 400° C....    | 72,000                   | 8                           | 140          | 36                        |
|         | 450° C....    | 85,000                   | 7                           | 171          | 49                        |
|         | 475° C....    | 88,000                   | 10                          | 171          | 53                        |
|         | 500° C....    | 89,000                   | 9                           | 171          | 56                        |
|         | 525° C....    | 85,000                   | 8                           | 168          | 57                        |
|         | 550° C....    | 81,000                   | 9                           | 158          | 60                        |
|         | 600° C....    | 73,000                   | 8                           | 128          | 55                        |
| 22----- | Cold drawn... | 67,000                   | 3                           | 128          | 24                        |
|         | Aged at:      |                          |                             |              |                           |
|         | 350° C....    | 65,000                   | 4                           | 130          | 29                        |
|         | 400° C....    | 69,000                   | 6                           | 138          | 38                        |
|         | 450° C....    | 85,000                   | 10                          | 174          | 51                        |
|         | 475° C....    | 87,000                   | 9                           | 179          | 58                        |
|         | 500° C....    | 88,000                   | 9                           | 171          | 62                        |
|         | 550° C....    | 79,000                   | 9                           | 158          | 65                        |
| 29----- | Cold drawn... | 66,000                   | 3                           | 124          | 26                        |
|         | Aged at:      |                          |                             |              |                           |
|         | 350° C....    | 65,000                   | 4                           | 120          | 29                        |
|         | 400° C....    | 72,000                   | 8                           | 138          | 39                        |
|         | 450° C....    | 85,000                   | 10                          | 163          | 54                        |
|         | 475° C....    | 87,000                   | 10                          | 174          | 60                        |
|         | 500° C....    | 90,000                   | 10                          | 169          | 63                        |
|         | 550° C....    | 74,000                   | 8                           | 153          | 65                        |
| 38----- | Cold drawn... | 67,000                   | 3                           | 126          | 20                        |
|         | Aged at:      |                          |                             |              |                           |
|         | 350° C....    | 65,000                   | 4                           | 133          | 24                        |
|         | 400° C....    | 70,000                   | 7                           | 143          | 30                        |
|         | 450° C....    | 91,000                   | 10                          | 177          | 39                        |
|         | 475° C....    | 94,000                   | 8                           | 182          | 44                        |
|         | 500° C....    | 92,000                   | 9                           | 180          | 47                        |
|         | 550° C....    | 92,000                   | 8                           | 170          | 51                        |

| Example   | Condition     | Tensile strength, p.s.i. | Elong., percent in 2 inches | Hardness VPN | Elec. cond., percent IACS |
|-----------|---------------|--------------------------|-----------------------------|--------------|---------------------------|
| 5 41----- | Cold drawn... | 69,000                   | 4                           | 123          | 22                        |
|           | Aged at:      |                          |                             |              |                           |
|           | 350° C....    | 70,000                   | 4                           | 134          | 26                        |
|           | 400° C....    | 74,000                   | 7                           | 143          | 33                        |
|           | 450° C....    | 88,000                   | 10                          | 177          | 43                        |
|           | 475° C....    | 91,000                   | 9                           | 177          | 47                        |
|           | 500° C....    | 91,000                   | 9                           | 174          | 52                        |
|           | 550° C....    | 89,000                   | 11                          | 165          | 53                        |
|           | 600° C....    | 73,000                   | 9                           | 140          | 50                        |

Having described my invention as related to the embodiments set out herein, it is my intention that the invention be not limited by any of the details of description, unless otherwise specified, but rather be construed broadly within its spirit and scope as set out in the accompanying claims.

I claim:

1. A copper base alloy having good responses to precipitation hardening and cold working consisting essentially of: about 0.4-1.5% chromium, about 0.3-0.9% titanium, about 0.1-0.8% nickel, about 0.02-0.16% phosphorus, and substantially the entire remainder a member of the class consisting of initially oxygen free and deoxidized copper, the amount ratio of nickel to phosphorus being about 5 of nickel to 1 of phosphorus and the amount of titanium being about 1-1.7 times the sum of the amounts of nickel plus phosphorus, the percentages and amounts being by weight.

2. The alloy of claim 1 precipitation hardened and cold worked to produce in the alloy high tensile strength, good electrical conductivity and excellent hardness.

3. The alloy of claim 1 in which the amount of chromium is about 1%.

References Cited

UNITED STATES PATENTS

|           |         |                |            |
|-----------|---------|----------------|------------|
| 1,991,162 | 2/1935  | Kroll          | 148—32.5 X |
| 2,189,198 | 2/1940  | Comstock       | 75—164 X   |
| 2,362,007 | 11/1944 | Hensel et al.  | 75—153 X   |
| 2,783,143 | 2/1957  | Johnson et al. | 75—164 X   |
| 3,162,529 | 12/1964 | Doi            | 75—164 X   |

FOREIGN PATENTS

45 120,469 10/1945 Australia.

CHARLES N. LOVELL, Primary Examiner.

U.S. Cl. X.R.

75—153, 164